

E. H. MEIGS.  
HAND AX.

No. 80,868.

Patented Aug. 11, 1868.



Fig. 1.



Fig. 2.



Witnesses.

E. H. Meigs  
J. W. Bays

Inventor.

E. H. Meigs

# United States Patent Office.

EDMOND H. MEIGS, OF EAST BERLIN, CONNECTICUT, ASSIGNOR TO ROYS, WILCOX, AND COMPANY, OF SAME PLACE.

*Letters Patent No. 80,868, dated August 11, 1868.*

## IMPROVED HAND-AXE.

The Schedule referred to in these Letters Patent and making part of the same.

TO ALL WHOM IT MAY CONCERN:

Be it known that I, EDMOND H. MEIGS, of East Berlin, county of Hartford, and State of Connecticut, have invented certain new and useful Improvement in the Manufacture of Hand-Axes; and, to enable others skilled in the art to make and use the same, I will proceed to describe its construction by referring to the drawings, in which the same letters indicate like parts in each of the figures.

The nature of this invention will be understood from the specifications and drawings, the object of which is to cheapen the manufacture, and produce a good article for use.

In the accompanying drawings—

Figure 1 is a side and edge view of an axe when finished.

Figure 2 is a side and edge view of an axe, as produced in the casting, before any work is wrought upon it; and also shows the shape and formation of the pattern used to form the mould in which the axe is cast, (except that it does not show the core front, which forms the edge of the axe.)

*a* is the body of an axe.

*c* is the eye of an axe.

*d* is a core-front piece, of cast steel, which, in the manufacture, is swaged into a uniform size and shape, to correspond with the print in the pattern, so that, when the mould is formed, and the pattern removed, the steel, *d*, may be placed therein, as shown in fig. 2.

*d'* are prints, or surplus amount of iron, just at the point where the iron and steel are to unite upon the surface of the metal. The object of this surplus iron at this point is to prevent it (the iron) from chilling, and, consequently, secure a perfect union of cast iron and steel, and produce a smooth united surface, without the use of any substance or material except the inherent property of the two metals, "cast iron and cast steel." The only preparation required is to have the surface of the steel perfectly cleansed on the sides which are desired to be united or welded to the cast iron.

The iron is poured into the mould in the usual way, and flowed across the steel, at the point of unity, into the mould, and into a pool formed in the flask just outside of the mould, to allow of a surplus flow of iron, to secure a welding-heat to the steel.

Thus it will be seen that, by this improvement, a cast-iron axe having a cast-steel edge can be produced, the two metals being firmly united together in the process of casting, and, when finished, which is done the common way, it has the appearance of a first-quality axe, formed of wrought iron and cast steel.

I believe I have thus shown the nature, construction, and advantage of this invention, so as to enable others skilled in the art to make and use the same therefrom.

I claim a hand-axe, produced substantially as described, as an improved article of manufacture.

E. H. MEIGS.

Witnesses:

E. W. BLISS,  
J. W. BLISS.